

Aug. 9, 1932.

R. H. MCKEE

1,871,419

PLIABLE HUMIDIFYING SHEET MATERIAL

Filed April 11, 1929



BY

INVENTOR  
RALPH H. MCKEE  
*A. Dr. Deller*  
ATTORNEY

## UNITED STATES PATENT OFFICE

RALPH H. MCKEE, OF JERSEY CITY, NEW JERSEY

## PLIABLE HUMIDIFYING SHEET MATERIAL

Application filed April 11, 1929. Serial No. 354,381.

The present invention relates to pliable humidifying sheet materials, and more particularly to pliable materials carrying humidifying agents in dry state and capable 5 of being placed in contact with articles which are to be maintained in a humid condition without being deleteriously affected thereby.

Heretofore articles or products such as cigarettes, cigars, candy edibles and the like 10 have been maintained in a moist condition by placing in the cabinet, show case, container or the like an absorbent containing water or any aqueous solution. Sometimes a sponge or a similar absorbent object was utilized 15 as a reservoir for holding water and giving it off to the surrounding environment as the latter tended to become dry. The use of liquids and wetted absorbents was objectionable, as is well known, and various 20 proposals were made to overcome the inherent disadvantages. Of these various proposals one of the more important was the suggestion of the utilization of divers organic and inorganic chemicals capable of 25 giving off water. These chemicals were filled into jars and other vessels which were placed in cabinets or show cases for preventing the atmosphere therein from becoming dry. The use of jars or the like was incon- 30 venient and some of the chemicals tended to dust off onto the articles being moistened and to give such articles a salt taste while some other chemicals tended to emit undesirable odors. For a variety of reasons, 35 consequently, the use of a mass of chemicals held in a vessel in open contact with the articles being preserved was objectionable. Attempts were made to overcome the shortcoming of the aforesaid proposals by providing 40 porous solid bodies which would absorb large quantities of water in a liquid condition in their pores. These porous bodies were damp and wet and were undesirable like wet sponges mentioned hereinbefore.

45 The aforesaid advantages are so serious that cigar manufacturers, for instance, have refused to sell retailers more cigars than can be sold within a relatively short period of time. If a retailer buys too large a supply, 50 the boxes of cigars stand on the shelf for so

long a time that the cigars tend to become dry and lose their quality. When dried cigars have been sold to the consuming public, the cigars have been unsatisfactory and have fallen into disfavor and the brands of those 55

cigars have a tendency to get a bad reputation. Manufacturers of cigars or the like have been faced with the aforesaid problem for a long time and in spite of the many proposals made to solve this problem, all attempts thus far made, as far as I am aware, has been unsatisfactory for one reason or other. Among the more important suggested proposals as noted hereinabove were absorbents and chemicals. Absorbents were intended, as is well known, to hold water in the liquid state and to give off the water vapor to the surrounding atmosphere. In addition to other objections, a humidor of the absorbent type could not be incorporated within a container such as a box of cigars. Chemicals, as mentioned heretofore, have been attempted to be used for maintaining the atmosphere within 60 cigar show cases or the like, in a humid condition by placing a mass of chemicals in an open jar or vessel which was positioned inside of the show case. In practice it was found that the chemicals tended to dust out of the jar into contact with the cigars or the like in the show case and thus spoil the 65 articles particularly by giving them a salty taste. The art consequently has never adopted chemical humidors particularly in close contact with cigars as inside of a cigar box. All prior efforts to provide individual humidor 70 for cigar boxes, as far as I am aware, have been unsatisfactory and unsuccessful.

75 I have invented a sheet material which carries humidifying agents in dry condition and which is capable of being wrapped about or of being placed in intimate and direct contact with cigars, cigarettes or other articles that are to be maintained in a humid state without deleteriously affecting the said articles. It is within the contemplation of my 80 invention to avoid all the disadvantages of prior humidifying means as noted hereinabove and to provide an improved humidifying material which is flexible or pliable, 85 which is sanitary, which is odorless and dry 90

to touch, and which is portable and dustless. My invention also contemplates the provision of a humidifying sheet material which is simple and economical to manufacture and 5 easy to use.

From the following description of a preferred embodiment of my invention other advantages and features will be apparent. In the drawing:

10 Fig. 1 is a plan view of a sheet of material embodying my invention, part of the sheet being turned to show the interior thereof;

Fig. 2 is a sectional view taken on the line 2—2 of Fig. 1;

15 Fig. 3 is a view similar to Fig. 2 of a modified embodiment of my invention; and

Fig. 4 represents a diagrammatic view of a container with a piece of my humidifying sheet material wrapped about articles which 20 are to be maintained in a moist condition, parts of the container and the sheet material being broken away to show the internal arrangement.

In the drawing the numeral 1 designates 25 a sheet of absorbent material preferably of a foraminous material or of a bibulous, fibrous nature like blotting paper. Within this absorbent material is incorporated a multiplicity of solid particles carrying water. Although a variety of materials may 30 be used as a humidifying agent for incorporation in material 1, I prefer to use an inorganic salt containing water of hydration such as Glauber's salt ( $Na_2SO_4 \cdot 10H_2O$ ).

35 The sheet material 1 containing a humidifying agent is preferably encased or enclosed completely within an envelope of flexible material which is capable of permitting the passage of water vapor from the absorbent material to the exterior and, at the same time, of preventing the passage of dust from the absorbent material. The envelope may be constituted of suitable material and made in an appropriate way. In Fig. 1 I have illustrated the envelope made of a rear portion 40 of tissue paper, muslin or fine cheese cloth with sealing margins 4 which can be united to the face of sheet material 1 such as by glue, paste or the like. The front portion of the 45 envelope is made by a cover 5 of tissue paper or fine meshed cloth which is sealed to the sheet material preferably at the margins or borders 4. Instead of this construction a regular tissue paper envelope can be used

50 in which sheet material 1 containing Glauber's salt or the like is placed. The flap of the envelope is used to seal the sheet material 1 within the envelope.

55 In the sheet material illustrated, the humidifying agent is Glauber's salt and is present in an amount of about two-thirds gram per square inch. The amount of humidifying material may, of course, be varied depending on the particular circumstances but 60 in practice I prefer to use a bibulous paper

capable of carrying upwards of about one-half a gram per square inch. For instance, a sheet of my material having a face about 8" by about 9" and being about  $\frac{1}{12}$ " thick, carries say 50 grams of Glauber's salt and 70 is suitable for use in humidifying a cigar box containing 50 cigars or a candy box of approximately the same size. If 50 grams of Glauber's salt ( $Na_2SO_4 \cdot 10H_2O$ ) is used, there are 28 grams of water potentially available for humidifying purposes. When the aforesaid sheet containing 50 grams of Glauber's salt is used with a cigar box having a 75 volume of about 1400 c. c. my humidifying sheet contains sufficient water vapor to 80 change the relative humidity within the box from approximately 15% to 60% about 2500 times. In other words, the box can be opened and closed about 2500 times without the 85 cigars drying out. Air, of course, is continually leaking in and out of the cigar box, and my humidifying sheet material automatically maintains the cigars and the interior of the box in a humid condition and 90 controls the moisture concentration in the cigar box as it stands on the dealer's shelves or as it is opened and closed.

An ordinary cigar carries from 0.25 gram to 1.00 gram of moisture depending upon its size and the character of the tobacco. Accordingly a container such as indicated hereinabove would be sufficient fully to take care of the moisture from a box of fifty cigars. Indeed it is far more than that because 95 the loss of moisture from the cigar occurs only when the air about it becomes dry, that is, of lower relative humidity.

100 In Fig. 3 a modified embodiment of my humidifying sheet material is illustrated which is constituted of an absorbent material 10 containing a humidifying agent 11. Upon each side of the material 10 a moisture pervious cover 12 is placed and secured. A preferred manner of securing cover 12 to sheet material 10 is to paste or glue the border about the periphery of said sheet material. In this way the absorbent material is practically completely sealed by the superposed covers 12. Except for the modifications my 105 humidifying sheet material is just the same as the form described in connection with 110 Figs. 1 and 2.

115 The humidifying agent, say Glauber's salt, is incorporated within the absorbent material by taking the blotting paper and passing it through a strong or an approximately saturated solution of the salt being used, allowing it to dry superficially and then wrapping it with tissue paper and pasting the tissue paper on the blotting paper so that it covers all edges. It is desirable in such a case to see 120 that the adhesive used is not used over the entire surface of the tissue paper but only on selected margins or lines. Otherwise the diffusion of moisture from the device to the 125

box in which it is located would be slowed down by the coating of nearly impervious adhesive.

It is to be observed that my invention provides a convenient dry sheet material which can easily and readily be wrapped about cigarettes in a package so as to keep them in a humid condition without deleteriously affecting them or used as a liner for bottom or sides 5 or both bottom and sides of a box containing cigars for the same purpose. My improved humidifying sheet material can also be used in closed show cases for covering the shelves, upon which boxes of cigars or other tobacco 10 products are placed, so as to maintain the show case in a humid condition and to prevent the cigars or other similar products from 15 drying out.

It is to be noted that instead of using Glauber's salt, sodium phosphate 20



or sodium carbonate ( $\text{Na}_2\text{CO}_3 \cdot 10\text{H}_2\text{O}$ ) may be employed. Glauber's salt gives a relative 25 humidity at temperatures normally prevailing within inhabited quarters of about 70%. Sodium phosphate gives a relative humidity of about 65% but after a loss of one fourth of its water it gives only 30 about 30%. Sodium carbonate gives a relative humidity of about 65% until nine-tenths of its water has been removed, and then a very much lower humidity.

I claim:

35 1. A flexible humidifying sheet material of "dry" character comprising a body of absorbent fibrous material having large face areas and having relatively thin edges, a multiplicity of dry solid chemical particles 40 incorporated in said fibrous material, and thin fibrous lining covering at least said two faces of said body of fibrous material and being pervious to moisture and impervious to dust of said chemical particles, said sheet material 45 being free from liquid water.

2. A flexible humidifying sheet material of "dry" character comprising a body of bibulous sheet material containing a humidifying agent in dry state capable of evolving 50 water vapor and an envelope of thin fibrous material encasing said body of sheet material and permitting the passage of water vapor but preventing the passage of dust, said sheet material being free from liquid water.

55 3. A pliable humidifying sheet material of "dry" character capable of being wrapped in direct contact with the article to be maintained in moist condition comprising a sheet blotting paper impregnated with dry Glauber's salt and a tissue paper envelope encasing 60 said blotting paper, said sheet material being free from liquid water.

4. A pliable humidifying sheet material of "dry" character capable of being wrapped in direct contact with the article to be main- 65

tained in moist condition comprising a sheet blotting paper having relatively large faces and a thin thickness and impregnated with Glauber's salt in an amount of about one half a gram of dry Glauber's salt per square inch 70 and a tissue paper envelope encasing said blotting paper, said sheet material being free from liquid water.

5. A flexible humidifying sheet material of "dry" character comprising a porous sheet 75 of paper fibers containing a dry, hydrated inorganic salt capable of evolving water vapor when placed in an atmosphere of low relative humidity, and a thin envelope of fine-meshed, fibrous material covering at least one side of 80 said porous sheet in such a manner as to permit the passage of water-vapor but to prevent the passage of salt dust, said sheet material being free from liquid water.

In testimony whereof I have hereunto set 85 my hand.

RALPH H. MCKEE.

90

95

100

105

110

115

120

125

130